



US005485181A

**United States Patent** [19]  
**Convers**

[11] **Patent Number:** **5,485,181**  
[45] **Date of Patent:** **Jan. 16, 1996**

[54] **INK JET PRINthead WITH IMPROVED DURABILITY**

4,509,063 4/1985 Sugitani et al. .... 346/140 R  
4,543,318 9/1985 Maeda et al. .... 430/288  
4,572,888 2/1986 Maeda et al. .... 430/288  
4,609,427 9/1986 Inamoto et al. .... 156/633  
4,956,035 9/1990 Sedlak .... 156/664  
5,019,483 5/1991 Lin et al. .... 430/288

[75] Inventor: **Ronald J. Convers**, Towanda, Pa.

[73] Assignee: **E. I. Du Pont de Nemours and Company**, Wilmington, Del.

[21] Appl. No.: **245,409**

*Primary Examiner*—Benjamin R. Fuller  
*Assistant Examiner*—Valerie Ann Lund

[22] Filed: **May 18, 1994**

[57] **ABSTRACT**

[51] **Int. Cl.<sup>6</sup>** .... **G01D 15/16**

Durability of ink jet printheads is improved by employing certain sulfur-containing adhesion promoters between the photoresist intermediate layer and the top plate having a noble metal surface.

[52] **U.S. Cl.** .... **347/63; 347/71; 347/65;**  
156/60

[58] **Field of Search** .... 347/63, 64, 65,  
347/71; 156/60

[56] **References Cited**

**U.S. PATENT DOCUMENTS**

3,617,411 11/1971 Coutore .... 156/307

**10 Claims, No Drawings**



-continued



6, 8-dithiooctanoic acid

(-S(CH<sub>2</sub>)<sub>n</sub>COOH)<sub>2</sub> where n is at least 1,

where n is at least 1,



where n is at least 1,



where m is at least 1, where n is at least 1, and where p is at least 1,

where m is at least 2, and where n is at least 2,  
4-(2-Thienyl)butyric acid and 6,8-dithiooctanoic acid are preferred, and are both available from Aldrich Chemical company, Milwaukee, Wis..

The amount of adhesion promoter is highly dependent on the adhesion promoter selected, and the reactive group present on the surface of the resin layer. The adhesion promoter typically is applied at a rate of 3 to 100 mg/cm<sup>2</sup>, preferably 3-50 mg/cm<sup>2</sup>. Higher amounts may be needed when the promoter is added to the resin layer instead of the top plate.

## TOP PLATE

The top plate is then bonded to the developed barrier material. The adhesion promoter may be applied to the top plate in a very thin uniform layer prior to bonding it to the resin layer or the top plate may be bonded to the adhesion promoter layer present on the resin layer. The top plate has a base plate and a surface layer of a noble metal. Some examples of noble metals include gold, platinum, palladium and iridium. Some examples of base plates include glass, ceramics, metal, plastics, thermoplastic resins such as acrylic resins, ABS resins, polyethylene and the like. Preferably the top plate is gold-surfaced.

## PROCESS

Details on how these general steps are accomplished will vary with the specific printhead design and manufacturer. In one embodiment, a noble metal-surfaced top plate may be washed with a dilute solution of the adhesion-promoting

compound to form a very thin layer, dried, aligned appropriately with features on the face of a bottom plate which bears printed microcircuits and an imaged and developed resin layer, and then bonded with the resist surface using heat and pressure. If more than a very thin, uniform coating is applied, deposits of adhesion promoter are formed which may interfere with the desired close contact of the resin layer to the noble metal surface, which is required if one end of an adhesion promoter molecule is to bond to the resist and the other end of the same molecule is to bond to the noble metal.

## EXAMPLES

The following examples, wherein parts and percentages are by weight, illustrate but do not limit the invention.

## EXAMPLE 1

Three approximately 2 cm×5 cm strips of a 30 micron thick coating of a photoresist or resin layer similar to that described in Example 7 of U.S. Pat. No. 4,937,172 on 0.92 mil (23.4 microns) polyethylene terephthalate film were given a UV photocure (75 mJ/cm<sup>2</sup>) and then laminated to the gold-plated surface of three 5 cm×5 cm plates using a Riston® hot roll laminator set at 100° C., 40 psig, and 1 meter/minute. The gold-plated surface of the first plate had previously received no adhesion promoter treatment, whereas the gold-plated surface of the second plate had been previously briefly immersed in a 1 weight percent solution of 4-(2-thienyl)butyric acid (Aldrich Chemical Company, Milwaukee, Wis.) in ethyl acetate and air-dried at room temperature. The gold-plated surface of the third plate had been treated with a 1 weight percent solution of thiocetic acid (Aldrich Chemical Company, Milwaukee, Wis.) in ethyl acetate and air-dried at room temperature. The resulting laminates were baked at 150° C. for 1 hour and cooled. The polyethylene terephthalate films were then peeled away and discarded. The resists were scored with a sharp knife in a cross-hatch pattern of approximately 5 mm×5 mm squares. Pieces of Scotch™ 810 tape were pressed firmly, with rubbing for 10 seconds, onto the cross-hatched surfaces of each of the three resists and then ripped away as quickly as possible from the resist surfaces. Again pieces of tape were pressed firmly, with rubbing for 10 seconds, onto the cross-hatched surfaces of the three resists and then ripped away as quickly as possible from the resist surfaces. If any resist was pulled away with the tape, the resist and/or the adhesion promoter were a failure. Failure tended to start with small chips of resist being removed by the tape from the edges of the cross-hatched cuts, i.e., a few percent of the resist-covered gold surface being re-exposed to view. Worse failure showed as larger areas of the resist-covered gold surface being re-exposed to view.

The sample having the untreated gold surface had only about 10-30 percent of the resist remaining on the gold surface after the tape test. With 4-(2-thienyl)butyric acid (Aldrich Chemical Company, Milwaukee, Wis.) as the adhesion promoter, no improvement was seen. However, with thiocetic acid (Aldrich Chemical Company) as the adhesion promoter, no edge chipping occurred. The results show that not all adhesion promoters are equally effective and that the choice of adhesion promoter is dependant on the composition of the resin layer.

## EXAMPLE 2

Example 1 was repeated with the following exceptions: a photoresist similar to that described in Example 10 of U.S.

Pat. No. 4,937,172 was used. The untreated sample showed better, but still insufficient gold adhesion with about 5 percent of the resist-covered gold surface being re-exposed to view in the tape test. Both 4-(2-thienyl)butyric acid and thiocetic acid treated samples displayed no edge chipping in the tape test.

### EXAMPLE 3

Example 2 was repeated with the following exceptions: a 0.10% solution of thiocetic acid in ethyl acetate was used instead of a 1% solution. The untreated control sample showed about 1-2 percent of the resist-covered gold surface reexposed to view after the tape test. The samples with the thiocetic acid treatment showed no edge chipping after the tape test.

What is claimed is:

1. In a printhead of an ink jet printer, said printhead comprising a top plate with a noble metal surface, an intermediate photoresist layer, and a bottom plate, the improvement wherein an adhesion promoter having the formula

$X(-R-Y)_n$ ,

wherein

X is a thioether, disulfide, polysulfide, or sulfur-containing heterocycle group;

Y is a terminal group that reacts with the photoresist;

R is a flexible non-polar molecular group; and

n is at least one;

is employed between said noble metal surface and said photoresist layer.

2. The printhead of claim 1 wherein the photoresist layer surface has epoxide reactive molecular groups.

3. The printhead of claim 2 wherein Y is selected from the group consisting of -OH, -NH, -SH, -COOH and carboxylic anhydride.

4. The printhead of claim 1 wherein said adhesion promoter is applied at a rate of approximately 3 to 100 mg/cm<sup>2</sup>.

5. The printhead of claim 1 wherein n is greater than one.

6. The printhead of claim 1 wherein R is a linear aliphatic chain.

7. The printhead of claim 1 wherein Y forms a covalent bond with reactive molecular groups on the photoresist layer.

8. The printhead of claim 7 wherein Y is selected from the group consisting of -OH, -NH, -SH, -COOH, carboxylic anhydride, reactive diene or dienophile, and a reactive unsaturated moiety.

9. The printhead of claim 1 wherein the adhesion promoter is 4-(2-thienyl)butyric acid.

10. The printhead of claim 1 wherein the adhesion promoter is 6,8-dithiooctanoic acid.

\* \* \* \* \*